

## UNITED STATES PATENT OFFICE

RALPH M. HUNTER, OF MIDLAND, MICHIGAN, ASSIGNOR TO THE DOW CHEMICAL COMPANY, OF MIDLAND, MICHIGAN, A CORPORATION OF MICHIGAN

METHOD OF PRODUCING SUBSTANTIALLY PURE METALLIC MAGNESIUM DIRECTLY BY ELECTROLYSIS OF A FUSED BATH

No Drawing.

Application filed May 31, 1929. Serial No. 367,251.

The present invention relates to the production of metallic magnesium by the electrolysis of a fused bath containing magnesium chloride.

5 An object of the invention is to separate the metal directly from the bath in a sufficiently pure condition to enable its use in the arts without further refining.

It has been considered necessary and has 10 been the practice heretofore, so far as I am aware, to subject metallic magnesium produced in the electrolytic process to a subsequent refining procedure. Various modes of such procedure have been used or proposed.

15 One of the least costly procedures is to remelt the crude metal in the presence of a limited amount of a suitable flux with which it is then agitated, said flux being of a character to coat the surface of the metal ex-

20 posed to the air so as to protect it from oxidation. After a period of such washing, the basic magnesium compounds present in the raw metal are largely washed out and transferred to the flux whereupon the metal may 25 be dipped or otherwise separated from the flux and cast into ingots or disposed of as desired.

Such practice requires a rehandling and remelting of the metal and provision of 30 associated plant and apparatus for the refining step.

I have invented a method of producing the equivalent of the so refined metal directly in the electrolytic cell whereby such rehandling, remelting and plant costs are saved.

To the accomplishment of the foregoing and related ends, the invention, then, consists of the method hereinafter fully described and particularly pointed out in the 40 claims, the following description setting forth in detail one mode of carrying out the invention, such disclosed mode illustrating, however, but one of various ways in which the principle of the invention may be used.

I electrolyze a suitable fused bath containing magnesium chloride and sodium chloride. The exact composition of the bath appears to be unimportant. Any bath suited to liberate magnesium upon electrolyzing 50 will serve as a washing agent in my process, as hereinafter described.

I prefer to use for the electrolysis a type of cell in which the liberated metal floats upon the bath. I prefer in any event a type 55 of cell in which the metal is gathered together into a compact molten mass. Such an electrolytic cell is disclosed in co-pending application Serial Number 210,785 by Louis E. Ward and the applicant herein. In the 60 cell therein described the metal is automatically led into a gathering or collecting well. Other forms of construction than 65 therein disclosed may obviously be employed, and it is further obvious that in some such, the collecting well or zone may be at one 70 side or one end, i. e. along the margin of the fused bath, thereby permitting easy access for the operations hereinafter described.

I permit the metal to collect in such well by the gathering together of the separate globules of metal preferably under restricted contact with the air or in an atmosphere of hydrogen, if the metal be floating upon the 75 bath, which latter gas may accompany the metal liberated due to the presence of water or basic chloride in the chloride fed to the bath. After the metal has collected to a substantial depth, which may be several 80 inches, I find that it has acquired a consistent character, the separate globules having coalesced and squeezed out the bath or flux. I agitate or mix it with the cell bath which may be readily done by removing the 85 cover above the metal, if one be used, inserting a ladle, dipping and pouring the metal over and over whereby it is contacted with the bath. Mechanical agitating means may, however, be employed, driven by power, if 90

desired, to impart relative motion to the bath and the metal whereby fresh surfaces of metal are brought successively into contact with the bath. After a short period of such 5 washing I withdraw the metal and cast it into molds. This may be done by ladling or other procedure convenient or desirable. I find the metal so treated before withdrawing from the cell to have substantially the same 10 degree of purity as the metal heretofore produced by withdrawing from the bath without such treatment, casting into crude ingots, subsequently remelting, washing with a flux and again casting into ingots. The 15 metal may be obtained by means of my simplified procedure with a purity of 99.85 percent or better.

The impurities in the metal are washed out by the bath, and inasmuch as such increment of impurity in the bath is a small one, substantially no additional burden is placed upon the dredging of the sludge from the cell incident to its normal operation.

Much effort has been directed to the development of the technical details of "after" 25 refining, i. e. remelting in a refining flux. The fused bath, which is used in the cell, may or may not have the ideal composition indicated by such research. I find, however, 30 that equivalent results are readily and cheaply obtained employing the cell bath itself as refining flux. "After" refining usually has been done by washing the remelted metal with a quite limited weight of flux,

35 whereas in my method I wash it with a relatively very large weight of flux. The use of flux to the extent of one-half (or less) the weight of metal is a customary ratio for "after" refining. In my method the weight

40 of the flux or bath relative to the metal may be several hundred times that of the latter. The dredging of the sediment is a normal operation in the electrolytic step which procedure keeps the bath effectively clean and 45 active as a washing agent for the metal. The advantage of a large ratio of flux to metal appears to outweigh any disadvantage which may be inherent in the bath composition relative to an ideal composition thereof.

50 In "after" refining the bath being small is rapidly fouled and must be discarded or returned to a larger molten mass for settling and reconditioning. In my method no such additional labor or procedure is required.

55 The bath has its cleansing power renewed automatically in the normal course of operation for the liberation of the metal.

The requirement for "after" refining has been based upon the fact that metallic magnesium heretofore obtained by electrolysis of a fused bath has shown a maximum purity 60 from 90 to 95 percent depending upon the type of cell used. I find that if the metal be gathered into a restricted area to a substantial depth enabling it to aggregate into

a consistent mass and be then washed, as herein described, the purification is unexpectedly improved and a metal in excess of 99 percent pure is readily obtained.

I find further that practicing washing upon such an aggregated mass of metal there results a prompt and effective separation of the metal from the flux and that the withdrawal of the metal from the cell with a minimum amount of flux, is easily done the total impurity including the flux being less than one percent of the total withdrawn.

70 Although my method of producing a substantially pure metal is more readily applicable when employed in large scale working i. e. with electrolytic cells using current in excess of 10,000 amperes, it may be employed in small scale production with advantage.

75 It is obvious that my improved method eliminates the requirement for separate melting pots, furnaces and associated equipment incident to and connected with "after" refining. It saves the cost of rehandling, labor and fuel for remelting. It also consolidates the production and refining steps at one point in one vessel requiring a minimum of supervision, labor, fuel and equipment and hence constitutes a valuable advancement in the art.

80 Other modes of applying the principle of my invention may be employed instead of the one explained, change being made as regards the method herein disclosed, provided the step or steps stated by any of the 90 following claims or the equivalent of such stated step or steps be employed.

85 I therefore particularly point out and distinctly claim as my invention:—

1. In a method of the character described, 100 the step which consists in washing molten metallic magnesium with the fused bath containing magnesium chloride from which it has been liberated by electrolysis before removal of said metal from said bath.

2. In a method of the character described, 110 the steps which consist in electrolyzing a fused bath containing magnesium chloride, gathering together the globules of the liberated metal into a consistent mass substantially free from inclusions of bath, agitating and washing the so gathered metal with the bath and removing the purified metal from the bath.

3. In a method of the character described, 120 the steps which consist in electrolyzing a fused bath containing magnesium chloride under conditions permitting the liberated metal to float thereon, gathering the liberated metal into a consistent mass floating on said bath, agitating and washing the so collected metal with the bath upon which it floats and removing the purified metal from the bath.

125 4. In a method of producing a substan-

tially pure magnesium metal by electrolysis of a fused bath containing magnesium chloride, the steps which consist in gathering together the globules of metal so liberated into a consistent mass substantially free from inclusion of bath and then setting up relative motion between said gathered metal and the bath whereby fresh surfaces of the metal are brought successively into contact with the bath.

Signed by me this 28th day of May, 1929.  
RALPH M. HUNTER.

15

20

25

30

35

40

45

50

55

60

65